

# UNITED STATES PATENT OFFICE.

ARTHUR EICHENGRÜN, OF ELBERFELD, GERMANY, ASSIGNOR TO FARBEN-FABRIKEN OF ELBERFELD CO., OF NEW YORK, N. Y., A CORPORATION OF NEW YORK.

## PROCESS OF DEVELOPING PHOTOGRAPHIC PICTURES.

SPECIFICATION forming part of Letters Patent No. 716,396, dated December 23, 1902.

Application filed December 17, 1901. Serial No. 86,305. (No specimens.)

*To all whom it may concern.*

Be it known that I, ARTHUR EICHENGRÜN, doctor of philosophy, chemist, residing at Elberfeld, Germany, (assignor to the FARBEN-FABRIKEN OF ELBERFELD Co., of New York,) have invented certain new and useful Improvements in Processes of Developing Photographic Pictures, of which the following is a specification.

As it is known, neutral and acid sulfites of alkalies are employed in photography as admixtures to the photographic developing-baths in order to prevent an oxidation of the developer which is employed; but the use of sulfites entails great inconveniences, inasmuch as their solutions cannot be kept and as the sulfites are decomposed by the action of the air. I have now found that these inconveniences in developing the photographic pictures can be obviated by employing instead of the above-mentioned sulfites the additive compounds obtained from ketones and bisulfites, especially the compounds which are prepared from acetone and potassium or sodium bisulfite, the so-called "acetone-alkali bisulfites" having the following general formula:



M meaning an alkaline metal, such as potassium or sodium. These additive compounds have the great advantage that they are readily soluble in water and that even their concentrated solutions keep long in a well-corked bottle without decomposing. On adding alkalies to the developing-baths containing acetone-alkali bisulfites the latter yield acetone,

which, as is known, has a very good influence on the developing process. Small quantities 40 of the acetone-alkali bisulfites suffice to render the developing-baths stable. For instance, the following formula may be employed with good result: one part of pyrogalol, one part of acetone-alkali bisulfite, six 45 parts of potassium carbonate, and one hundred parts of water.

Having thus described my invention and in what manner the same is to be performed, what I claim as new, and desire to secure by 50 Letters Patent, is—

1. The herein-described process of developing photographic pictures consisting in subjecting them to the action of a photographic developing-bath containing additive compounds from ketones and bisulfites, substantially as described.

2. The herein-described process of developing photographic pictures consisting in subjecting them to the action of a photographic developing-bath containing acetone-alkali bisulfite having the formula



65

M having the hereinbefore-defined meaning, substantially as described.

In testimony whereof I have signed my name in the presence of two subscribing witnesses.

ARTHUR EICHENGRÜN.

Witnesses:

OTTO KÖNIG,  
J. A. RITTERSHAUS.